

Patented Oct. 31, 1933

1,933,068

# UNITED STATES PATENT OFFICE

1,933,068

## DYEING FIBROUS MATERIAL

Joseph Nuesslein, Ludwigshafen-on-the-Rhine, Germany, assignor, by mesne assignments, to General Aniline Works Inc., New York, N. Y., a corporation of Delaware

No Drawing. Original application October 16, 1925, Serial No. 62,932, and in Germany October 30, 1924. Divided and this application August 19, 1929. Serial No. 387,088

8 Claims. (Cl. 8—5)

The present invention relates to dyeing of fibrous materials and this application has been divided out from my copending application Ser. No. 62,932 filed October 16th, 1925.

5 I have found that the treatment of fibrous materials with dyeing liquors is considerably improved if the dyeing liquors are prepared with an addition of a small quantity of sulfonic acids of such aromatic hydrocarbons as contain alkyl 10 groups with more than two carbon atoms, especially of naphthalene and similar hydrocarbons with several benzene rings containing propyl or butyl (normal or iso) groups.

The term fibrous materials is employed in a 15 broad way including all textile fibres, for example wool, cotton, natural and artificial silk and the like, also jute, straw, paper, leather, hides, furs, feathers and the like, and the dyeing process is the usual one which is carried out in a dyeing 20 liquor as contrasted with the little usual dyeing in the lather.

The said sulfonic acids enable the fibrous materials to be wetted very rapidly in an excellent manner and make it unnecessary to apply any 25 special boiling operation to the goods before introducing them into the dyebath. The said sulfonic acids have the advantage of being insensitive to acids or hard water. Consequently they can be employed not only in alkaline or 30 neutral dyebaths but also in acid baths. In any case, very uniform dyeings are produced even with dyestuffs which make this very difficult when dyed in the usual way.

The sulfonic acids may be employed as such 35 or in the state of their salts. Sometimes it may be advantageous to use the free sulfonic acids or their salts in mixture with aliphatic alcohols, especially the higher members of this group that is to say such as contain more than 3 carbon 40 atoms.

The following examples will more fully explain the manner of carrying the invention into practice which, however, I do not wish to limit in any way to these examples. The numbers 45 after the trade names of the dyestuffs employed correspond to those of the Color Index, 1st edition, 1924.

### Example 1

50 A piece of woollen cloth is introduced into a lukewarm dyebath prepared from 0.6 per cent of cyananthrol BGA, (1077) 0.6 per cent of azoflavine FDN, (147) 0.2 per cent of sorbire red, (54) 10 per cent of Glauber's salt, 2 to 3 per 55 cent of sulfuric acid of 66 degrees Baumé and 2

per cent of isopropylated naphthalene sulfonic acid sodium salt, and stirred for about 10 minutes. The bath is then heated to the boil in the course of  $\frac{1}{4}$  to  $\frac{1}{2}$  hour and after being kept boiling for one hour, it is allowed to cool. The 60 goods are then well rinsed.

Or the goods, for example hats in a half planked state, carbonized or impure, are wetted in the evening before dyeing by handling for half an hour at 70 degrees Centigrade in a bath 65 containing 0.5 per cent of isopropylated naphthalene sulfonic acid sodium salt, left in the bath during the night and dyed in the next morning in the above described manner with an addition of 0.5 per cent of the said sulfonic acid 70 sodium salt, 20 per cent of Glauber's salt and the necessary quantity of acid to the dyebath.

If instead of the sodium salt the free sulfonic acid is employed, the sulfuric acid may be left out wholly or partly. 75

### Example 2

Unboiled, raw cotton yarn is directly introduced at 50° to 60° C. into a dyebath containing 10 per cent of indanthrene blue RS (1106) 80 and, in each litre, 12 cubic centimetres of caustic soda lye of 40 degrees Baumé, 1.5 grams of dry sodium hydrosulfite and 2 to 4 grams of isopropylated naphthalene sulfonic acid sodium salt, dyed for  $\frac{3}{4}$  to 1 hour as usual with indanthrene dyestuffs and finished by rinsing and soaping in a boiling bath. 85

### Example 3

Unboiled, raw cotton yarn is directly introduced into a boiling dyebath prepared from 3 per cent of oxamine blue B (515) and, in each litre, 10 grams of Glauber's salt and 1 to 3 grams of isopropylated naphthalene sulfonic acid sodium salt. The goods are dyed for 1 hour 90 in the manner usual for direct dyestuffs and finished as usual.

The developing of dyestuffs on the fibrous materials may be effected in a similar manner.

Instead of the sodium salt of isopropylated 100 naphthalene sulfonic acid, other soluble salts or the free acid or butylated naphthalene sulfonic acid or their salts may be employed.

What I claim is:—

1. As new articles of manufacture aqueous 105 preparations suitable for dyeing comprising a vatted vat dyestuff and an aromatic sulphonic acid containing an alkyl radicle with more than two carbon atoms.

2. As new articles of manufacture aqueous 110

preparations suitable for dyeing comprising a vatted vat dyestuff of the indanthrene series and an aromatic sulphonic acid containing an alkyl radicle with more than two carbon atoms.

5 3. As new articles of manufacture aqueous preparations suitable for dyeing comprising a vatted vat dyestuff, a reducing agent and an aromatic sulphonic acid containing an alkyl radicle with more than two carbon atoms.

10 4. As new articles of manufacture aqueous preparations suitable for dyeing comprising a vatted vat dyestuff, a reducing agent, alkali and an aromatic sulphonic acid containing an alkyl radicle with more than two carbon atoms.

15 5. As new articles of manufacture aqueous preparations suitable for dyeing comprising a vatted vat dyestuff and a naphthalene sulfonic acid containing an alkyl radicle with more than two carbon atoms.

20

6. As new articles of manufacture aqueous preparations suitable for dyeing comprising a vatted vat dyestuff, a naphthalene sulphonic acid containing an alkyl radicle with more than two carbon atoms, and an aliphatic alcohol containing more than 3 carbon atoms in its molecule.

7. As new articles of manufacture aqueous preparations suitable for dyeing comprising a vatted vat dyestuff and a propylated naphthalene sulphonic acid.

8. As new article of manufacture an alkaline aqueous preparation suitable for dyeing comprising water, about 10 per cent its weight of a vatted dyestuff of the indanthrene series and about 0.3 per cent its weight of a propylated naphthalene sulphonic acid.

JOSEPH NUESSLEIN.

80

85

90

95

25

100

30

105

85

110

40

115

45

120

50

125

55

130

60

135

65

140

70

145

75

150